

# United States Patent

Huber-Emden et al.

[15] 3,679,779

[45] July 25, 1972

## [54] PHOSPHONIC ACID DIALKYL ESTERS

[72] Inventors: **Helmut Huber-Emden; Karl Eschle**, both of Basel; **Arthur Maeder**, Therwil, all of Switzerland

[73] Assignee: **Ciba-Geigy AG**, Basel, Switzerland

[22] Filed: **Jan. 22, 1970**

[21] Appl. No.: **5,148**

## [30] Foreign Application Priority Data

Jan. 30, 1969 Switzerland ..... 1460/69

[52] U.S. Cl. ..... **260/943, 117/136, 260/45.9 R,**  
260/562 A, 260/562 B, 260/562 S, 260/969

[51] Int. Cl. ..... **C07f 9/40**

[58] Field of Search ..... 260/943

## [56] References Cited

### UNITED STATES PATENTS

2,875,232 2/1959 McConnell et al. .... 260/943 X  
2,908,605 10/1959 Beriger et al. .... 260/943 X

Primary Examiner—Joseph Rebold

Assistant Examiner—Richard L. Raymond

Attorney—Harry Goldsmith, Joseph G. Kolodny and Mario A. Monaco

[57]

## ABSTRACT

The subject of the invention is phosphonic acid dialkyl esters of the formula



in which R denotes an alkyl radical with one to 18 carbon atoms and n denotes 1 or 2. These phosphonic acid dialkyl esters are used as antioxidants for plastics, especially for polypropylene, polyethylene and polyurethane, and rubber. The combined use of the phosphonic acid dialkyl esters with flameproofing agents, may increase the flameproofing action of the flameproofing agent. The use of the compounds according to the invention in combination with other antioxidants also may show advantageous effects.

10 Claims, No Drawings

## PHOSPHONIC ACID DIALKYL ESTERS

The subject of the invention is phosphonic acid dialkyl esters of formula



wherein R denotes an alkyl residue with one to 18 carbon atoms and n denotes 1 or 2.

Preferred phosphonic acid dialkyl esters correspond to the formulas



wherein R1 denotes an alkyl residue with 12 to 18 carbon atoms and n denotes 1 or 2, and also



wherein R2 denotes an alkyl residue with two to four carbon atoms and n denotes 1 or 2.

Amongst the compounds encompassed by formulas (2) and (3), those of formulas



wherein n denotes 1 or 2 and



wherein n denotes 1 or 2, are above all of interest. The compound of formula



is particularly suitable.

The phosphonic acid dialkyl esters of formula (1) are thus for example dimethyl, diethyl, dibutyl, didodecyl or dioc-tadecyl esters. Depending on whether n is 1 or 2, different starting products are used for the manufacture of these dialkyl esters.

If n = 1, the procedure followed is that, in accordance with the principle of the Michaelis-Arbusow reaction, (a) a compound of formula



wherein Y denotes a halogen atom, is condensed with (b) a compound of formula



5 wherein R denotes an alkyl residue with one to 18 carbon atoms. This reaction can be carried out without solvents or in a suitable solvent, such as for example xylene. The halogen atom Y in the formula (7) can for example represent an iodine or bromine atom or especially a chlorine atom.

10 The starting product of formula (7) required for this reaction is obtained from 2,6-di-tertiary-butylphenol and N-methylol-chloracetamide by Tscherenik condensation. This latter reaction is known and is described in French Pat. Specification No. 1,571,696.

15 The compounds of formulas (2), (3), (4) and (5) with n = 1 are accordingly obtained by using, as component (b), a compound of formulas



25 wherein R1 and R2 have the indicated significance.

Phosphonic acid dialkyl esters of formula (1), wherein n = 2, are manufactured by reacting (a) a compound of formula



35 with (b) a compound of formula



40 wherein R represents an alkyl residue with one to 18 carbon atoms. This reaction is approximately carried out in an anhydrous medium, for example a suitable organic solvent such as absolute dioxan, tetrahydrofuran or 1,2-dimethoxy-ethane. The reaction is catalysed by the presence of small amounts of sodium salt of the corresponding compound of formula (14), which is first formed in situ by the addition of metallic sodium.

45 The starting product of formula (13) required for this reaction can be obtained from 2,6-di-tertiary-butylphenol and N-methylol-acrylamide by Tscherenik condensation in glacial

50 acetic acid in the presence of pyrophosphoric acid, as has already been described in French Pat. Specification 1,475,097.

A more rational route for the manufacture of the compound of formula (13) consists in the same reaction except for the

55 pyrophosphoric acid being replaced by gaseous hydrogen chloride. In this, a 1:1 addition product of the compound of formula (13) and N-(3,5-di-tertiary-butyl-4-hydroxyphenyl-methyl)-β-chloropropionamide first precipitates directly:



65 The compounds of formula (13) is obtained in good yields from the addition product of formula (15) by splitting off HCl by means of sodium hydrogen carbonate.

The compounds of formulas (2), (3), (4) and (5) with n = 2 are accordingly obtained by using, as component (b), a com-

70 pound of one of the formulas





wherein  $\text{R}_1$  and  $\text{R}_2$  have the indicated significance.

The phosphonic acid dialkyl esters of formulas (1) to (6) are used as antioxidants for plastics. Possible plastics are polyethylene, polyurethane and above all polypropylene; further, also polyvinyl chloride and rubber.

When protecting oxidation-sensitive plastics against oxidation, the appropriate procedure is to incorporate into these plastics a small amount, preferably 0.01 to 2 percent relative to the amount of plastic to be protected, of at least one compound of formulas (1) to (6).

The compounds of formula (1) can for example be worked into the plastics to be protected directly, that is to say by themselves or together with other additives such as plasticizers, pigments, light protection agents, fluorescent whitening agents, flameproofing agents or other antioxidants, and/or with the aid of solvents.

The combined use of the compounds of formulas (1) to (6) together with flameproofing agents, especially those containing phosphorus, shows certain advantages, above all in polyurethane coating compositions. This is because in addition to the actual antioxidant action, the compounds of formulas (1) to (6) are also able distinctly to increase the flameproofing action of the flameproofing agent.

The use of the compounds of formulas (1) to (6) in combination with other antioxidants, namely carboxylic acid amides containing sulphur, have proved particularly advantageous.

These carboxylic acid amides are known from French Pat. Specification 1,571,696 and correspond to the formula



wherein  $\text{R}_1$  denotes a benzene residue which carries a hydroxyl group in the o-position or p-position to the  $-\text{CH}_2-$  group and carries two hydrocarbon residues as further substituents,  $\text{R}_2$  denotes a hydrogen atom, an alkyl or aryl residue which is optionally substituted further, or a residue of formula



wherein  $\text{R}_1$  has the indicated significance and  $m$  denotes an integer having a value of at most 2, and  $n$  denotes an integer having a value of at most 7. Carboxylic acid amides of formula (20), wherein the residue  $\text{R}_2$  carries several thioether residues, are preferred. In particular, thioethers of formulas



have proved particularly advantageous in combination with the phosphonic acid alkyl esters of formulas (1) to (6).

The quantity ratio of the phosphonic acid dialkyl esters of formula (1) and the sulphur-containing carboxylic acid amides of formula (20) in combination preparations varies within wide limits. Preparations which contain 20 percent by weight of a compound of formula (20) and 80 percent by weight of a compound of formula (1) have for example proved advantageous.

In general, the combination preparations show a better antioxidant action than the individual components alone.

In the manufacturing instructions and examples which follow, percentages are percentages by weight.

#### MANUFACTURING INSTRUCTIONS

5 51.5 g of 2,6-di-tertiary-butylphenol and 26.5 g of N-methylolacrylamide are successively dissolved in 50 ml of glacial acetic acid with gentle warming. Thereafter HCl gas is introduced whilst stirring, and with exclusion of moisture, until saturation is reached. The reaction is exothermic; the temperature is kept at 30°C by external cooling.

During the reaction a thick precipitate forms. Thereafter the mixture is stirred for a further 3 to 4 hours at room temperature and then for a further one-half hour at 5 to 10°C.

15 The product is then thoroughly suction-filtered off and rinsed with a little glacial acetic acid. The filter residue is stirred with 1 liter of water, filtered off and rinsed with water. 57.7 g (=75 percent of theory) of the 1:1 addition product of N-(3,5-di-tertiary-butyl-4-hydroxyphenyl-methyl)-acrylamide and N-

20 (3,5-di-tertiary-butyl-4-hydroxy-phenyl-methyl)- $\beta$ -chloropropionamide are obtained; melting point: 168° to 171°C. This product can be recrystallized from acetone or chloroform without decomposition and without change in melting point.

25 An aqueous suspension of this product initially reacts neutral, but reacts acid after a short time.

The 1:1 addition product together with 16.8 g of sodium hydrogen carbonate and 200 ml of acetone is boiled for 1 hour under reflux whilst stirring. The mixture is cooled, undissolved

30 inorganic material is filtered off and the solvent is removed in vacuo. The oily residue rapidly crystallizes throughout after seeding. 54 g of N-(3,5-di-tertiary-butyl-4-hydroxyphenyl-methyl)-acrylamide of melting point 107 to 109°C, corresponding to formula (13), are obtained.

35 The product is recrystallized from 400 ml of cyclohexane and 47.1 g (=65 percent of theory, relative to the 2,6-di-tertiary-butylphenol employed) of the acrylamide of melting point 112° to 113°C are obtained.

40 The acrylamide of formula (13) can also be obtained in almost quantitative yield from the 1:1 addition products by vigorously stirring the latter with excess 2N sodium carbonate solution for several hours and washing the product, after filtering off the sodium carbonate solution, until a neutral reaction is obtained; melting point: 110° to 111.5°C. When manufactured according to this latter method, the substance is not entirely free of bonded chlorine.

#### EXAMPLE 1

50 18 g of N-(3,5-di-tertiary-butyl-4-hydroxyphenylmethyl)-chloracetamide are dissolved in 50 ml of dry xylene by warming. 7.22 g of phosphorus acid trimethyl ester are added and the mixture is heated to gentle boiling under reflux. The reaction is complete when the reaction solution contains no

55 further bonded chlorine, which can easily be followed by occasional sampling and testing by means of the Beilstein reaction. Gentle boiling under reflux for 40 to 45 hours suffices.

Thereafter the mixture is cooled, whereupon the product precipitates after a short time. 16.2 g (=73 percent of theory) of a compound of melting point (after recrystallization from benzene or from xylene) 142° to 143°C are obtained, corresponding to the formula



#### EXAMPLE 2

An analogous procedure to example 1 is followed, using phosphorous acid triethyl ester (instead of the trimethyl ester)

in the stoichiometric amount. Yield: 62 percent of theory; melting point (after recrystallization from xylene or cyclohexane): 97° to 99° C. The compound corresponds to the formula



## EXAMPLE 3

18 g of N-(3,5-di-tertiary-butyl-4-hydroxyphenylmethyl)-chloracetamide and 14.6 g of phosphorous acid tributyl ester are heated together for 2 hours to 175° C (bath temperature) in a reflux apparatus, with an air condenser. During the course of this, nitrogen is passed into the reaction vessel in order to expel the resulting butyl chloride through the reflux condenser. Thereafter the mixture is cooled and recrystallized from 80 ml of cyclohexane. 20 g (=73 percent of theory) of a compound of formula (26) are obtained.

A larger sample is chromatographically purified on silica gel using an ascending eluent series of benzene-chloroform, and is then again recrystallized from cyclohexane; melting point: 91° to 92° C.



## EXAMPLE 4

9 g of N-(3,5-di-tertiary-butyl-4-hydroxyphenyl-chloracetamide and 17 g of phosphorous acid tridodecyl ester are heated in a distillation apparatus with a stirrer, at 15 mm Hg pressure, for 2 hours with stirring to 175° C, finally reaching 200° C (bath temperature). In the course thereof, 3.75 g (=63 percent of theory) of dodecyl chloride distil off at 135° to 148° C.

After cooling, the residue is chromatographed on silica gel with an ascending eluent series of benzene-chloroform, whereupon 15 g (=75 percent of theory) of a waxy-crystalline product of melting point 47° to 49° C are obtained, corresponding to the formula



## EXAMPLE 5

a. 9 g of N-(3,5-di-tertiary-butyl-4-hydroxyphenylmethyl)-chloracetamide and 24 g of phosphorous acid trioctadecyl ester are heated for 1½ hours in a distillation apparatus at 0.001 mm Hg pressure to 175°—185° C. (bath temperature), while stirring. In the course thereof, octadecyl chloride distils off, contaminated by a little N-(3,5-di-tertiary-butyl-4-hydroxyphenylmethyl)-chloracetamide, which under these conditions partially sublimes off.

The distillation residue is recrystallized from acetone and then from petroleum ether, whereupon the desired product of formula (28) is produced as a crystal mass resembling a hard wax; melting point: 71.5° to 72.5° C.



b. 9 g of N-(3,5-di-tertiary-butyl-4-hydroxyphenylmethyl)-chloracetamide and 25 ml of dry xylene are heated for 90 hours under reflux in nitrogen at a bath temperature of 175° C. Thereafter the solvent is removed in vacuo and the waxy residue is purified as described in example 5 a); melting point: 71.5° to 72.5° C.

Purification can also be effected by chromatography on silica gel with an ascending eluent series of benzene-chloroform-ethyl acetate.

10 The compound of formula (28) is obtained.

## EXAMPLE 6

27.6 g of phosphorous acid diethyl ester are dissolved in 150 ml of absolute dioxan. 0.5 g of sodium are added and the mixture is stirred for 15 hours under nitrogen. In the course thereof, the sodium dissolves and a small amount of a flocculent precipitate is produced.

57.8 g of N-(3,5-di-tertiary-butyl-4-hydroxyphenylmethyl)-acrylamide are now added; this dissolves rapidly and the mixture is stirred for a further 25 hours under closed condition. The solvent is then completely removed in vacuo. The resinous residue is recrystallized from dry benzene and the crystalline product is dried for some time in vacuo. 55.7 g (≈65 percent of theory) of the product of melting point 104 to 106° C are obtained, corresponding to the formula



35

## EXAMPLE 7

7.76 g of phosphorous acid dibutyl ester are dissolved in 30 ml of absolute dioxan. 0.1 g of sodium are added and the mixture is stirred under nitrogen for 15 hours; in the course thereof, the sodium dissolves and a small amount of a flocculent precipitate is produced. 11.57 g of N-(3,5-di-tertiary-butyl-4-hydroxyphenylmethyl)-acrylamide are now added and dissolve rapidly. Thereupon the reaction mixture, contained in a closed vessel, is stirred for 3 days, and is thereafter heated for a further 2 hours to the boil under reflux, in nitrogen.

The solvent is now completely removed in vacuo and the waxy-crystalline residue is recrystallized from cyclohexane. 12.6 g (≈65 percent of theory) of the compound of melting point 113° to 116° C are obtained, corresponding to the formula



60

## EXAMPLE 8

17.6 g of phosphorous acid dioctadecyl ester are dissolved in 100 ml of absolute 1,2-dimethoxyethane whilst warming. 70 mg of sodium are added and the mixture is heated for 18 hours under reflux in nitrogen, while stirring. In the course thereof, the sodium dissolves and a small amount of a flocculent precipitate forms. 8.67 g of N-(3,5-di-tertiary-butyl-4-hydroxyphenylmethyl)-acrylamide are added thereto; this dissolves rapidly and the mixture is heated for 24 hours under reflux in nitrogen.

Thereafter it is left to stand for 2 days at room temperature under closed conditions, whereupon a large part of the product crystallises out. Crystallizes further proportion is obtained by concentrating the mother liquor.

Purification is effected by recrystallization from a large amount of petroleum ether. 15.3 g (=58 percent of theory) of the compound of melting point 76° to 78° C, corresponding to formula (31), are obtained.

It is also possible to dissolve the crude product in chloroform and then to purify it by chromatography on silica gel. Hereupon, the substance is obtained as a chloroform adduct; melting point 35° to 36° C, the product resolidifies on further heating and finally melts at 72° to 74° C. The chloroform can be eliminated from this adduct by heating in a high vacuum (at 160° C/10 minutes/0.001 mm Hg.).



### EXAMPLE 9

A mixture of 20 percent of the thioether of formula (22) or (23) and 80 percent of the phosphonic acid dialkyl ester of formula (27) is heated with stirring, under a nitrogen atmosphere, for 1 minute to 130° or 165° C respectively, whereupon cloudy to clear melts are produced. The mixture is then quenched by cooling with cold water.

The following combinations were obtained according to this process:

TABLE I

| Mixture | Thioether of formula | Phosphonic acid dialkyl ester of formula | Consistency |
|---------|----------------------|------------------------------------------|-------------|
| A (22)  |                      | (27)                                     | Resinous    |
| B (23)  |                      | (27)                                     | Resinous    |

### TEST OF ANTOXIDATIVE EFFECTIVENESS

A mixture of 100 parts of unstabilized polypropylene and 0.2 part of a phosphonic acid dialkyl ester of formula (1) or of their combination products with thioethers of formula (20) is processed on a calender at 170° C to give a hide. This is then pressed at 230° C and a pressure of 40 kg/cm<sup>2</sup> to give a 1 mm thick sheet. The sheet is cut into narrow strips and is left to age in an oven at 140° C until distinct cracks can be detected visually.

The results are summarized in table II. For comparison, the ageing times achievable with the thio compounds of formula (22) or (23) alone are also given. It can be seen from the figures that the combination of the phosphonates with the thio compounds give even better protection against ageing than the individual compounds alone.

TABLE II

| Added compound of formula, or combination | Time to crack formation, in hours |
|-------------------------------------------|-----------------------------------|
| Without additive                          | 5                                 |
| (25)                                      | 35                                |
| (26)                                      | 75                                |
| (27)                                      | 600                               |
| (28)                                      | 1000                              |
| (29)                                      | 25                                |
| (30)                                      | 60                                |
| (31)                                      | 530                               |
| (22)                                      | 500                               |
| (23)                                      | 600                               |
| A                                         | 1100                              |
| B                                         | 1000                              |

### EXAMPLE 10

Mixtures of 100 parts of rubber (latex crêpe), 5 parts of zinc oxide, 10 parts of titanium dioxide, 75 parts of barium sulphate, 1 part of stearic acid, 1.5 parts of 2-mercaptobenzothiazole, 2 parts of sulphur and 1 part of one of the compounds of formulas (25), (26), (27), (30), (31) or of

combination B (see example 9) are homogeneously mixed on a two-roll mill at 60° C for 30 minutes and subsequently pressed to give 1 mm thick sheets by vulcanization for 20 minutes in a press at 140° C. Dumb-bell-shaped 8 cm long pressed specimens are punched from these and are then aged for 50 hours in an oven at 100° C. The decrease in the mechanical strength and the antioxidant action of the abovementioned compounds can be recognized by measuring the breaking load and elongation at break before and after ageing.

The results are summarized in table III. The figures given are in each case average values from 5 tests at a time.

In table III the symbols denote:

L = breaking load in kp/mm<sup>2</sup>  
D = elongation at break in %

TABLE III

| 20 | Antioxidant of<br>Mechanical<br>formula, or<br>combination | oven ageing, 100° C<br>hours | Decrease<br>in % |             |
|----|------------------------------------------------------------|------------------------------|------------------|-------------|
|    |                                                            |                              | 0                | 50          |
| 25 | Without<br>additive                                        | L<br>D                       | 1.29<br>910      | 1.03<br>772 |
|    | (25)                                                       | L<br>D                       | 1.52<br>976      | 1.36<br>814 |
|    | (26)                                                       | L<br>D                       | 1.32<br>934      | 1.21<br>800 |
|    | (27)                                                       | L<br>D                       | 1.51<br>1012     | 1.33<br>877 |
| 30 | (30)                                                       | L<br>D                       | 1.48<br>932      | 1.39<br>802 |
|    | (31)                                                       | L<br>D                       | 1.24<br>930      | 1.1<br>772  |
|    | B                                                          | L<br>D                       | 1.31<br>944      | 1.18<br>824 |
|    |                                                            |                              |                  | 10<br>12.7  |
| 35 |                                                            |                              |                  |             |

### EXAMPLE 11

100 parts of polyethylene granules are mixed dry with 0.2 part of one of the compounds of formulas (25), (26), (27), (28), (29), (30), (31) or of combinations A or B, and are subsequently processed on a two-roll mill at 140° C for 3 minutes to give a homogenous hide. This is then pressed in a press at 150° C for 5 minutes to give an 0.2 mm thick foil. The dumb-bell-shaped 8 cm long test specimens required for the tear tests are punched therefrom and are then aged for 200 hours in an oven at 85° C. The decrease in mechanical strength and the antioxidant action of the abovementioned compounds can be recognized by measuring the breaking load and elongation at break.

The results are summarized in table IV. The values given are in each case average values from 5 samples at a time.

The symbols denote:

L = breaking load in kp/mm<sup>2</sup>  
D = elongation at break in %

TABLE IV

| 60 | Antioxidant of<br>Mechanical<br>formula, or<br>combination | Oven ageing, 85° C<br>hours | Decrease<br>in % |             |
|----|------------------------------------------------------------|-----------------------------|------------------|-------------|
|    |                                                            |                             | 0                | 200         |
| 65 | Without<br>additive                                        | L<br>D                      | 1.38<br>370      | 1.06<br>248 |
|    | (25)                                                       | L<br>D                      | 1.44<br>397      | 1.32<br>380 |
|    | (26)                                                       | L<br>D                      | 1.43<br>392      | 1.30<br>379 |
|    | (27)                                                       | L<br>D                      | 1.56<br>440      | 1.34<br>399 |
| 70 | (28)                                                       | L<br>D                      | 1.39<br>381      | 1.18<br>327 |
|    | (29)                                                       | L<br>D                      | 1.5<br>433       | 1.21<br>378 |
|    | (30)                                                       | L<br>D                      | 1.45<br>428      | 1.21<br>346 |
|    | (31)                                                       | L<br>D                      | 1.46<br>407      | 1.16<br>330 |
| 75 | A                                                          | L<br>D                      | 1.54<br>451      | 1.29<br>333 |
|    |                                                            |                             |                  | 16<br>26    |

|   |   |      |      |     |
|---|---|------|------|-----|
| B | L | 1.41 | 1.36 | 3.5 |
|   | D | 407  | 407  | -   |

## EXAMPLE 12

100 parts of polyethylene powder are mixed dry with 0.2 part of one of the compounds of formulas (25), (26), (27), (28), (29), (30) or of combinations A or B and subsequently processed for 3 minutes on a two-roll mill at 110° C to give a homogeneous hide. This is then pressed in a press at 130° C for 3 minutes to give a 1 mm thick sheet which is aged for 72 hours in an oven at 85° C. For determining the melt index, the sheets aged in this way are comminuted into small chips. The melt index is determined according to ASTM D-1238-62 T, method E (weight 2.16 kg, temperature 190° C, time 10 minutes). The increase in the melt index and the antioxidant action of the abovementioned compounds can thus be recognized. The results are summarized in table V.

TABLE V

| Antioxidant of formula or combination | Melt index in grams<br>Oven ageing, 85° C<br>hours | 0     | 72 |
|---------------------------------------|----------------------------------------------------|-------|----|
| -                                     | 3.525                                              | 5.121 | 25 |
| (25)                                  | 3.828                                              | 4.827 |    |
| (26)                                  | 3.934                                              | 4.560 |    |
| (28)                                  | 3.749                                              | 4.992 |    |
| (29)                                  | 3.937                                              | 4.903 |    |
| (30)                                  | 3.930                                              | 4.927 | 30 |
| A                                     | 3.741                                              | 4.831 |    |
| B                                     | 3.749                                              | 4.802 |    |

## EXAMPLE 13

5 percent of the compound of formula (25) or (29) or of the mixture consisting of 1 part of one of these compounds and 9 parts of commercially available flameproofing agent of formula bis-(2-hydroxy-ethyl)-amino-methane-phosphonic acid diethyl ester are stirred into a polyurethane coating composition of 20 g of isocyanate-modified polyester, 1 g of reaction accelerator, 1 g of polyfunctional isocyanate as a crosslinking agent and 5 ml of ethyl acetate. These mixtures are applied as a thin layer (0.5 mm) on flameproof cotton fabric by means of a doctor blade and cured in air at room temperature. The test specimens manufactured in this way are subjected to the flame test according to DIN 53906, oven ageing at 85° C and exposure to light in the Xeno test.

It can be seen from the results of table VI that an admixture of the compounds of formulas (25) or (29) to the flameproofing agent considerably increases its flameproofing action.

TABLE VI

| Additive to Flame test polyurethane according to coating com- DIN 53,906 position                                      | Oven ageing, Exposure to light 85°C/85 hours | in Xeno test for 20 hours |
|------------------------------------------------------------------------------------------------------------------------|----------------------------------------------|---------------------------|
| Without Burns very additive vigorously 5% of bis-(2-hydroxy-ethyl-amino-methane-phosphonic acid diethyl ester (= FSM)) | Trace yellow                                 | Colorless                 |
| 4.5% FSM + 0.5% of the Self-extinguishing formula (25)                                                                 | very yellow                                  | Yellowish                 |
|                                                                                                                        | Trace yellow                                 | Colorless                 |
|                                                                                                                        | yellow                                       |                           |

|                                                        |        |           |
|--------------------------------------------------------|--------|-----------|
| 4.5% FSM + 0.5% of the Self-extinguishing formula (25) | Trace  | Colorless |
|                                                        | yellow |           |

We claim:  
1. A phosphonic acid dialkyl ester of the formula



15 in which R is an alkyl radical with one to 18 carbon atoms and n is 1 or 2.

2. A compound according to claim 1 in which R is an alkyl radical with 12 to 18 carbon atoms.

20 3. A compound according to claim 1 in which R is an alkyl radical with two to four carbon atoms.

4. A compound according to claim 1 in which R is  $-\text{C}_{18}\text{H}_{37}$ .

5. A compound according to claim 1 in which R is  $-\text{C}_4\text{H}_9$ .

6. The compound according to claim 1 of the formula



7. The compound according to claim 1 of the formula



40 8. The compound according to claim 1 of the formula



50 9. The compound according to claim 1 of the formula



60 10. The compound according to claim 1 of the formula



\* \* \* \* \*